

[54] **PROCESS FOR PREPARING CRYSTALLINE SODIUM NITRILOACETIC ACID**[75] Inventors: **Robert B. Agee, Baker; William R. Cooke, Baton Rouge, both of La.**[73] Assignee: **Ethyl Corporation, Richmond, Va.**[22] Filed: **Dec. 7, 1970**[21] Appl. No.: **95,540**[52] U.S. Cl. .... **260/534 E**[51] Int. Cl. .... **C07c 101/20**[58] Field of Search ..... **260/543 E; 23/295**[56] **References Cited**

## UNITED STATES PATENTS

|           |         |               |        |
|-----------|---------|---------------|--------|
| 3,218,133 | 11/1965 | Ebner .....   | 23/295 |
| 3,399,976 | 9/1968  | Randolph..... | 23/295 |

## OTHER PUBLICATIONS

Bamforth "Industrial Crystallization", Leonard Hill (1965) pp. 156-167.

*Primary Examiner—Lorraine A. Weinberger**Assistant Examiner—John F. Terapane**Attorney—Donald L. Johnson, John F. Sieberth, Sheldon B. McAnelly and Arthur G. Connolly*[57] **ABSTRACT**

It is disclosed that the particle size distribution of crystalline sodium nitrilotriacetate (NTA) can be controlled to achieve a desired bulk density of the product and to provide a product that centrifuges readily. The control is obtained by conducting the crystallization and/or crystal growth of NTA in the presence of a centrifugal impeller operative at a peripheral velocity of from about 20 to about 80 feet per second whereby the crystals are selectively abraded or fractured to limit growth of the periphery of the crystals enhancing the relative growth rate of the crystals in the thickness dimension.

**14 Claims, 1 Drawing Figure**

Patented Sept. 11, 1973

3,758,565



## PROCESS FOR PREPARING CRYSTALLINE SODIUM NITRILOACETIC ACID

### BACKGROUND OF THE INVENTION

#### 1. Field of the Invention

This invention relates to the preparation of crystalline sodium nitrilotriacetate (NTA) by recovery from a supersaturated solution.

#### 2. Description of the Prior Art

Several processes are available for recovering solid NTA from an aqueous solution thereof. One such process is by crystallization from a supersaturated solution followed by separation of the resulting crystals in a centrifugal device to recover the crystals substantially free of mother liquor. It is characteristic of such crystallization that crystals formed are thin platelets which are characterized by a low bulk density of the recovered crystal product and by difficulty of separation of the crystals from the mother liquor in centrifugal devices because the crystals interweave. These characteristics are not significantly altered even with slow growth to comparatively large crystals or by other variations of the rate of crystal growth through such expedients as temperature and concentration variations of the growing solution because the ratio of crystal thickness to maximum periphery is unimpeded crystal growth is substantially constant.

### SUMMARY OF THE INVENTION

It has been discovered that an improvement is possible in the growth of NTA crystals to produce thicker crystals having a larger numerical ratio of thickness to periphery than that characterized by ordinary growth by mechanically agitating the mixture of growing crystals and accompanying mother liquor. With the proper severity of agitation as defined herein, the crystals are broken in a plane parallel to the thickness dimension without serious abrasion of the thickness dimension or retardation of the growth in the thickness dimension. The result is that the crystals are allowed to build up selectively in the thickness dimension with growth in directions at right angles to the thickness dimension being hindered. The product from such a crystallization operation, although frequently apparently smaller in size than the ordinary product when measured on a basis of mesh screens, centrifuges readily and has a desirable high bulk density of the order of 0.5 to 0.8 grams per cc.

Controlled manipulation of the crystals in the growth process is preferably accomplished with an agitation device which provides a moderate degree of shear. A centrifugal pump of conventional design with closed or open impeller when operated at certain speeds is an example of such a moderate shear agitation device. When such a pump is operated within the crystal growing system using peripheral velocities of the pump impeller of from about 20 to about 80 feet per second, desirable results with respect to control of the size and shape of the product trisodium nitrilotriacetate (NTA) are obtained. In this connection, it is noteworthy that the intimacy of contact attainable with a centrifugal impeller is apparently an important factor since other types of pumps commonly encountered such as the axial flow propeller type wherein the flow is primarily axial rather than centrifugal, do not produce the presently desired results even when operated at the upper regions of the peripheral velocities recited in the foregoing. On the

other hand, gear type and similar positive displacement pumps, even when operated at low speeds, exert a crushing and grinding action between internal surfaces providing generally a locally excessive comminution action.

Although the preferred manner of use of the centrifugal impeller is within a centrifugal pump (or a turbine pump) housing in a piped recirculation system, the present desired results are also obtained when such an impeller is merely inserted into a mass of concentrated aqueous NTA solution and NTA crystals and rotated so as to provide the specified peripheral velocities. In general, simple propeller type agitators inserted within the mass provide an equivalent of axial flow rather than centrifugal or radial flow and do not provide the presently desired results in a satisfactory manner.

The present invention relates to a process for producing solid particulate NTA of high bulk density by crystallization from a supersaturated aqueous solution of NTA favorable to the growth of thin platelet NTA crystals. The system of supersaturated solution and crystals is mechanically agitated, while the crystals are growing, by circulation through a centrifugal impeller operative at a peripheral velocity of from about 20 to about 80 feet per second whereby the crystals are selectively abraded or fractured to effectively limit growth of the periphery of the crystals enhancing the relative growth rate of the crystals in the thickness dimension.

In preferred aspects, the centrifugal impeller peripheral velocity is from about 40 to about 70 feet per second, a more preferred range being from about 45 to about 55 feet per second. By way of illustration, a typical peripheral velocity of the centrifugal impeller is about 50 feet per second.

In a preferred aspect, the centrifugal impeller is the impeller of a centrifugal pump disposed within a pump housing forming a pump which is interconnected by way of piping whereby the entire volume of the system of supersaturated aqueous solution of NTA and NTA crystals circulates through the pump in a period of from about 0.5 to about 5 minutes. A typical volumetric flow circulation rate for the system through the pump is an average of about once every 2 minutes.

In a preferred aspect of the process of the present invention, the system of NTA solution and NTA crystals is maintained at a temperature of from about 120° to about 250°F. A more preferred temperature range is from about 150° to about 200°F, or even from about 175° to about 195°F. A typical preferred temperature is 195°F. A typical temperature in accordance with the present invention is about 190°F.

In a preferred aspect, the process of the present invention grows NTA crystals in a system consisting essentially of an aqueous solution of NTA in admixture with from about 5 to about 50 wt. percent NTA crystals. In a more preferred aspect of the present invention, the crystal growing is conducted in a system which consists essentially of an aqueous solution of NTA and from about 20 to about 40 wt. percent NTA crystals. A typical system consists essentially of a mixture of an aqueous solution of NTA with about 35 wt. percent NTA crystals and from about 1 to about 5 percent NaOH copresent.

The present process produces solid particulate NTA of high bulk density and controlled particle size and shape by crystallization from an aqueous solution which contains from about 5 to about 50 wt. percent

NTA crystals in addition to at least a saturation amount of NTA at the temperature of operation which is from about 120° to about 250°F. Preferably, the solution is formed by the evaporation of water from a feed solution which is somewhat less than saturated. The foregoing solution is agitated with a centrifugal impeller operative at a maximum peripheral velocity of from about 20 to about 80 feet per second whereby the growing crystals are selectively abraded.

The present invention provides a process for producing solid particulate NTA of high bulk density and controlled particle size and shape wherein the NTA is crystallized from a solution. An important aspect of the process for the purpose of controlling particle size and shape is the recirculation of a system consisting essentially of an aqueous solution of NTA containing from about 5 to about 50 wt. percent free NTA crystals in a heater-flash evaporator wherein the system is alternately heated to a temperature of about 200°F and flashed at a temperature of about 195°F whereby water vapor is removed. Feed to the system is an NTA solution consisting essentially of from about 30 to about 40 wt. percent NTA and water. The recirculation of the process is conducted in two streams including (1) a low shear stream operative at a volumetric flow rate per minute of from about 1 to about 10 times the volume of said system, and (2) a moderate shear stream containing a centrifugal pump operative at an impeller peripheral velocity of from about 20 to about 80 feet per second and at a volumetric flow rate per minute of from about 0.2 to about twice the volume of said system.

The present invention provides a process for the concurrent concentration and crystallization of a solution of NTA ranging from about a saturated solution to a more dilute solution containing about 5 percent of the saturation amount of NTA. In the process there is performed a concurrent evaporation of water to form a chemical system containing a solution of NTA, usually supersaturated, and in addition, from about 5 to about 50 percent by weight of NTA crystals. The growth of crystals within the system is selectively controlled by a deliberate abrading or fracturing of the crystals by a centrifugal impeller operative within the system at a selected peripheral velocity. In a particularly preferred aspect, the present invention is performed in a mechanical system whereby the chemical system described in the foregoing is repetitively recirculated through a heater and a flash chamber by means of a pump at a rate from about 1 to about 10 times per minute.

In preferred embodiments of the present invention, in addition to the recirculation loop described in the foregoing, there is provided a second loop through a pump containing a centrifugal impeller operative at a peripheral velocity of from about 20 to about 80 feet per second through which the volumetric contents of the system flows in a period of from about 0.5 to about 5 minutes. In preferred embodiments, the first mentioned pump is a low shear axial flow pump with a propeller type agitator and the centrifugal impeller pump is a centrifugal pump of conventional design with closed impeller or open impeller construction.

An innovation of the process of the present invention is the deliberate operation of an agitator element within a crystallization system at a speed which is intended to cause controlled breaking of the crystals in the system.

The process of the present invention has been employed with centrifugal impeller pumps of various sizes ranging from a 4½ inch diameter impeller operative at 2,700 rpm providing 53 feet per second peripheral velocity to a 10½ diameter impeller pump operative at a speed of 1,900 rpm to provide 87 feet per second peripheral velocity. Larger and smaller diameter impellers are operated at proportionate speeds to attain the peripheral velocities set forth. Excellent operation is obtained with the 10½ inch diameter impeller operative at a speed of 1,160 rpm providing 53 feet per second peripheral velocity of the impeller. Throughput rate is determined in a conventional way involving proportioning of the diameter, speed, shape and thickness of the impellers. Where desired, increased flows are obtained without increased diameters of peripheral speeds by paralleling one or more impellers.

Direct measurement of throughput rate is not conveniently accomplished when the centrifugal impeller is located in the open in a large vessel. In this instance the actual flow across the impeller generally is of larger volume with less severity per unit of volume passing through the impeller. Also the horsepower requirements may increase.

It is evident that the procedures described herein provide a basis for routine experimentation to "tailor make" the particle size, shape and bulk density of the product NTA using either the direct agitation or separate pump approach.

With reference now to the drawing, the apparatus shown therein includes a flash chamber 10, typically operative at a temperature of 195°F and a pressure of about one-half atmosphere absolute. Steam flashed in the flash chamber 10 passes to condenser 11 where it is condensed and removed as water through line 12 with non-condensables flowing through line 13 to a vacuum system 14.

The flash chamber 10 is connected to a first recirculation loop of line 15, pump 16, heater 17 and lines 18, 19 and 20. This first recirculation loop is proportioned primarily to provide the desired heat input to the system for evaporation of water with a controlled warmup of about 4° to 6°F in the heater 17. In general, this requires a flow rate in the first recirculation loop of from about 1 to about 10 times the liquid volume of the system per minute, typically about 2 times the volume circulated per minute. The pump 16 is designed to provide the high flow rate at low head since the total head required to be produced by that pump is mainly only that introduced by friction in the lines 15, 18, 19 and 20 and in the heater 17. Typically, this pump is an axial flow pump with a "propeller" type of impeller similar to those used in marine service. In many instances these pumps attain peripheral velocities of 20-80 feet per second; however, the flow is rapid and much of the material flows through slower moving portions of the impeller. Thus this contact is not adequate for the purposes of the present invention. In fact, such pumps may be deliberately designed and operated to avoid breaking or abrading the crystals. Such pumps are of low shear type under the normal operating conditions employed.

A second recirculation loop is provided within the system employing the pump 21 and the connecting line 22 together with one or more of the alternate connecting lines 23 and 25. The recirculating pump 21 typically is a pump of a type which is considerably different

from pump 16 in that it is operated to produce a moderate shear action and is suitably of less volumetric throughput capacity than pump 16. Pump 21 contains a centrifugal impeller operative at a peripheral velocity of from about 20 to about 80 feet per second with a volumetric flow rate of from about 0.2 to about twice the volume of said system per minute, typically about 0.5 volume of the system per minute. The alternate discharge lines 23 and 25 for pump 21 provide for convenience of connection or to permit adding the volume of pump 21 to the volume of pump 16 for the feed through heater 17. In general, the discharge of the pumps 16 and 21 are advantageously combined for feed through the heater 17 in those instances where flow rate through pump 21 is greater than about half that of the flow rate through pump 16.

Feed to the system is provided at any convenient point, typically to line 15 between the flash chamber 10 and the pump 16. The feed preferably is an NTA solution which is about saturated containing about 1 percent residual sodium hydroxide, a characteristic of a preferred method of production of the feed stream which is typically by reaction of nitrilotriacetonitrile with a slight excess of caustic (NaOH) in an aqueous system. The presence of the caustic in the present system is of no major significance with respect to the overall principles of operation, the major effect being that of producing a reduction in the solubility of NTA in water. In general, the feed may range from a saturated solution of NTA upwards to more concentrated systems including solutions containing more than a saturation amount of NTA and, downward on the other hand, to solutions containing 5 percent or less (total) NTA by weight. In general, one prefers to pre-concentrate extremely dilute NTA solutions in a preceding evaporator to maintain a fairly constant typical concentration of NTA in the feed ranging from about 30 to about 40 percent NTA by weight.

Effluent is removed from the system at any convenient point, typically from the lines 19 or 20 or directly from the liquid of flash chamber 10. For simplicity and ease of control, the rate of withdrawal of the product is governed by the rate required to maintain a constant level within flash chamber 10 as sensed and regulated by level control 28.

Product removed through line 27 contains on a weight percent basis from about 30 to about 35 percent NTA crystals and from about 65 to about 70 percent mother liquor, the mother liquor containing at least a saturation amount of NTA of about 33 percent, plus about 5 percent sodium hydroxide and about 62 percent water.

The feed and effluent rates are typically proportioned, together with the liquid volume of the system, to provide an average NTA particle retention time in the system of about one hour with a convenient average circulation through pump 21 of about 30 times. Although this volume is preferred for convenience and economy of construction, suitable results are obtained with the average residence time ranging from about 5 minutes to about 10 hours with average circulation ranging from about 5 to about 100 times.

Although the two-pump scheme of the Figure is preferred because of the ability to separately control the circulations for evaporation and for crystal size control, it is possible to operate with a single centrifugal or "turbine" pump rather than with two pumps. The approach

to the problem in such instances is to design for the impeller peripheral speed indicated for crystal size control and to use an impeller vane width which provides an acceptable flow rate for acceptable heat input.

Although the flow through a separate heater 17 is generally preferred in a crystallization system to minimize fouling of heat exchanger surfaces and obtain good heat transfer, in appropriate instances the use of a separate heat exchanger may be unnecessary in which instance the pump 16 and the separate heater 17 are omitted. Where such is the case it is preferred to use the crystal control loop with its separate pump 21 designed for flow rates and peripheral speeds as set forth in the foregoing. Alternately, the centrifugal or "turbine" impeller of pump 21 may be inserted directly into the liquid mass in chamber 10 which may or may not operate as a flash chamber. In this instance, the impeller is operated at a peripheral speed as indicated in the foregoing and the thickness or diameter of the impeller or impellers is proportioned to achieve the desired control. In such instances, a first approximation for design is to use the same horsepower input for operation of the direct impeller as used in operation of a separate pump 21.

The following examples indicate preferred embodiments of the present invention.

#### EXAMPLE I

Apparatus was set up as in the Figure but without pump 21. Pump 16 was a centrifugal pump with a diameter of 11 $\frac{1}{2}$  inches operative at 1,160 rpm providing a peripheral velocity of 53 feet per second. The temperature of the flash chamber 10 was 181.5°F. The heatup through heater 17 was 3.5°F. The discharge through valve 27 contained 32 wt. percent NTA particles. The feed rate provided an average solids (NTA crystals) residence time of 0.85 hours.

The product centrifuged well, providing recovered NTA crystals  $[N(CH_2COONa)_3H_2O]$  of a bulk density of 0.68 containing 6-8 wt. percent moisture.

#### EXAMPLE II

Example I was repeated using a pump speed of 795 rpm providing a peripheral velocity of 40 feet per second. The temperature of the flash chamber 10 was 180.5°F, the heatup through heater 17 was 3.0°F. The discharge through valve 27 contained 27.6 wt. percent NTA particles. The feed rate provided an average solids residence time of 1.08 hours.

The product centrifuged well providing recovered NTA crystals of a bulk density of 0.66 containing 6-8 wt. percent moisture.

#### EXAMPLE III

Example I was repeated using a pump speed of 795 rpm providing a peripheral velocity of 40 feet per second. The temperature of flash chamber 10 was 196°F, the heatup through heater 17 was 3.5°F. The discharge through valve 27 contained 32.4 weight percent NTA particles. The feed rate provided an average solids residence time of 1.2 hours.

The product centrifuged well providing recovered NTA crystals of a bulk density of 0.65 containing 4 percent water.

#### EXAMPLE IV

Example I was repeated using a pump speed of 795

rpm providing a peripheral velocity of 40 fps. The temperature of the flash chamber 10 was 195°F, the heatup through heater 17 was 3°F. The discharge through valve 27 contained 27.6 wt. percent NTA particles. The feed rate provided an average solids residence time (NTA) of 1.25 hours.

The product centrifuged providing recovered NTA crystals of a bulk density of 0.6 containing 6-9 wt. percent moisture.

#### EXAMPLE V

Example I was repeated using a pump speed of 635 rpm providing a peripheral velocity of 32 fps. The temperature of the flash chamber 10 was 161°F, the heatup through heater 17 was 4.0°F. The discharge through valve 27 contained 27.0 wt. percent NTA particles. The feed rate provided an average solids (NTA particles) residence time of 1.2 hours.

The product centrifuged but not as well as in Examples I-IV. Recovered NTA had a bulk density of 0.55 and contained 10-12 wt. percent moisture.

#### EXAMPLE VI

Example I was repeated using a pump speed of 450 rpm providing a peripheral velocity of 22 feet per second. The temperature of the flash chamber was 183°F, the heatup through heater 17 was 4°-6°F. The discharge through valve 27 contained 24.2 wt. percent NTA particles. The feed rate provided an average solids (NTA particles) residence time of 0.9 hours.

The product would not centrifuge.

A sample of the product was obtained by filtration and other procedures. The bulk density was 0.5.

#### EXAMPLE VII

Foregoing examples were repeated with a centrifugal pump having a 4½ inch diameter impeller operative at 2,700 rpm providing 53 feet per second peripheral velocity. Desirable results similar to those of Examples I-IV were obtained.

#### EXAMPLE VIII

Foregoing examples were repeated in several examples with a centrifugal pump having a 10½ inch diameter impeller operative at 785, 1,160 and 1,900 rpm, providing, respectively, 36, 53, and 87 feet per second peripheral velocity.

Operation at 53 feet per second provided superior results with respect to ease of centrifuging, thoroughness of centrifuging, and bulk density of product.

#### EXAMPLE IX

Apparatus was set up as in the Figure, with pumps 16 and 21. Pump 21 discharged to the junction of lines 18 and 19. The liquid content of the system was 13 gallons. The feed rate was 162 lbs/hour. The product rate was 119 lbs/hours (slurry containing 30 percent by weight of NTA crystals) providing an average particle residence time in the system of 1.3 hours.

Pump 16 was a centrifugal pump having a 13 inch diameter impeller driven at a speed of 369 rpm providing a peripheral velocity of 21 feet per second. The flow through this pump was 18 gals./min., approximately 140 percent of the system volume per minute.

Pump 21 was a centrifugal pump having a 6 inch diameter impeller driven at a speed of 1,875 rpm providing a peripheral velocity of 49 feet per second. The

flow through this pump was 7 gallons per minute, approximately 54 percent of the system content per minute.

The product from the system centrifuged readily providing a particulate NTA product having a bulk density of 38.7 lbs./ft<sup>3</sup> with the following distribution:

- 3 percent on 30 mesh
- 42 percent on 50 mesh
- 85 percent on 100 mesh
- 10 98 percent on 200 mesh

#### EXAMPLE X

Example IX was repeated except pump 21 was inoperative. Other flow rates, through pump 16, feed and product, were the same. The product centrifuged poorly providing a product bulk density of 32.9 lbs/ft<sup>3</sup> with the following distribution:

- 15 percent on 30 mesh
- 72 percent on 50 mesh
- 95 percent on 100 mesh
- 98.5 percent on 200 mesh

We claim:

1. In a process for producing solid particulate NTA of high bulk density by crystallization in a system containing growing crystals of NTA in a supersaturated aqueous solution of NTA, the improvement wherein said solution and the crystals of NTA contained therein are circulated through a centrifugal impeller operative at a peripheral velocity of from about 20 to about 80 feet per second whereby the crystals are selectively abraded or fractured to limit growth of the periphery of the crystals enhancing the relative growth rate of the crystals in the thickness dimension.

35 2. The improvement of claim 1 wherein the temperature is from about 120° to about 250°F, and wherein the centrifugal impeller is the impeller of a centrifugal pump.

3. A process for producing solid particulate NTA of 40 high bulk density which comprises, forming a system containing a mixture of growing crystals of NTA and an accompanying supersaturated aqueous mother liquor solution, said system containing from about 5 to about 50 percent by weight of crystals of NTA, mechanically 45 agitating said system while the crystals are growing by circulation thereof through a centrifugal impeller providing a moderate degree of shear operation at a peripheral velocity of from about 20 to about 80 feet per second whereby the crystals formed are selectively abraded.

50 4. The process of claim 3 wherein the centrifugal impeller peripheral velocity is from about 40 to about 70 feet per second.

5. The process of claim 3 wherein the centrifugal impeller peripheral velocity is from about 45 to about 55 feet per second.

60 6. The process of claim 3 wherein the centrifugal impeller is in a pump housing and the entire volume of said system circulates through the pump housing in a period of from about 0.5 to about 5 minutes.

7. The process of claim 6 wherein the circulation of the entire system through the pump housing is an average of about once every 2 minutes.

65 8. The process of claim 3 wherein the solution temperature is from about 120° to about 250°F.

9. The process of claim 3 wherein the solution temperature is from about 150° to about 200°F.

10. The process of claim 3 wherein the solution temperature is from about 175° to about 195°C.

11. The process of claim 3 wherein the solution temperature is about 195° F.

12. The process of claim 3 wherein the system contains from about 20 to about 40 wt. percent NTA crystals.

13. The process of claim 3 wherein the system contains about 35 wt. percent NTA crystals.

14. A process for producing solid particulate NTA of high bulk density and controlled particle size and shape wherein the NTA is crystallized from a solution, which comprises:

recirculating a system consisting essentially of an aqueous solution of NTA and from about 5 to 15 about 50 wt. percent NTA crystals in an evaporator system wherein the system is alternately heated to

a temperature of about 200°F and flashed at a temperature of about 195°F whereby water vapor is removed,

feeding make-up NTA solution to said system consisting essentially of from about 30 to about 40 wt. percent NTA and water,

said recirculating being in two streams including (1) a low shear stream operative at a mass flow rate per minute of from about one to about 10 times the volume of said system and (2) a moderate shear stream containing a centrifugal pump operative at an impeller peripheral velocity of from about 20 to about 80 feet per second and at a mass flow rate per minute of from about 0.2 to about twice the volume of said system.

\* \* \* \* \*

20

25

30

35

40

45

50

55

60

65

UNITED STATES PATENT OFFICE  
CERTIFICATE OF CORRECTION

Patent No. 3,758,565 Dated September 11, 1973

Inventor(s) Robert B. Agee and William R. Cooke

It is certified that error appears in the above-identified patent and that said Letters Patent are hereby corrected as shown below:

Column 4, line 7, reads "imepll-", should read  
-- impell--. Column 10, line 10, reads "sheat", should  
read -- shear --.

Signed and sealed this 5th day of March 1974.

(SEAL)

Attest:

EDWARD M. FLETCHER, JR.  
Attesting Officer

C. MARSHALL DANN  
Commissioner of Patents